

May 17, 1966

H. S. SPACIL

3,251,684

METHOD OF FORMING COHERENT METALLIC MEMBERS

Filed Oct. 22, 1965



Inventor:  
Henry S. Spacil,  
by Paul R. Neff, II  
His Attorney.

1

3,251,684

## METHOD OF FORMING COHERENT METALLIC MEMBERS

Henry S. Spacil, Schenectady, N.Y., assignor to General Electric Company, a corporation of New York  
Filed Oct. 22, 1965, Ser. No. 507,609  
8 Claims. (Cl. 75—200)

This application is a continuation-in-part of my copending application filed January 2, 1963, as Serial No. 249,070, and assigned to the same assignee as the present application.

This invention relates to methods of forming coherent metallic members and more particularly to methods of forming coherent metallic members from metallic halides.

A method of producing iron powder is set forth in United States Letters Patent, 2,418,148, Williams et al., wherein ferrous chloride, which is maintained below its melting point, is subjected to hydrogen. Another method of forming iron powder is described in United States Letters Patent 2,663,633, wherein gaseous ferrous chloride, which is maintained above its melting point, is subjected to hydrogen. In United States Letters Patent 2,664,352, Darner et al., production of iron powder is described wherein ferrous chloride in liquid form is sprayed into a chamber into which hydrogen is introduced.

In each of the above patents, a method is disclosed for producing iron powder which powder must be subsequently processed by conventional techniques to produce useful coherent articles or shapes. It would be desirable to produce coherent metallic members by the reduction of their respective metallic halides. Such a method would be advantageous in providing directly the coherent metallic member. The present application is directed to methods of forming coherent metallic members by reduction from their respective metallic halides.

It is an object of my invention to provide coherent metallic members.

It is another object of my invention to provide a coherent metallic member from its respective metallic halide.

It is another object of my invention to provide a coherent metallic member from a mixture of metallic halides.

It is a further object of my invention to provide a coherent metallic member from at least one mixed metallic halide.

It is a further object of my invention to provide a coherent metallic member containing at least one inert non-metallic filler material.

It is a still further object of my invention to provide a coherent metallic member containing at least one inert metallic filler material.

In carrying out my invention in one form, a method of forming a coherent metallic member comprises forming at least one metallic halide powder into a preshaped powder member, positioning the preshaped member within a chamber, introducing into the chamber a stream of gas consisting essentially of hydrogen, and heating the member to a temperature in a temperature range having a lower limit in a range determined by the hydrogen halide partial pressure to the hydrogen partial pressure ratio in equilibrium with the metal of the member and with the member in a range from 0.001 to 0.01, and an upper limit in a range determined by the metallic halide vapor pressure multiplied by the number of halide atoms per metallic atom in a range from 0.001 to 0.01 whereby the member is reduced to a coherent metallic member.

These and various objects, features and advantages of the invention will be better understood from the follow-

2

ing description taken in connection with the accompanying drawing in which:

The single figure of the drawing is a graph plotting the standard free energy of formation of metallic chlorides per mole of chlorine in kilocalories versus temperature in degrees centigrade.

The present invention is directed to methods of forming coherent metallic members by the reduction of their respective halides under specific conditions. Nickel, cobalt, chromium, silver, copper and iron are produced from their respective halides. Various alloys are also formed by appropriate mixtures of the respective metallic halides. For example, nickel-copper, nickel-chromium, nickel-chromium-iron, iron-chromium, iron-nickel-chromium, iron-nickel-cobalt, iron-cobalt, iron-nickel, copper-nickel-iron, and copper-nickel-cobalt, are produced by this method.

I discovered unexpectedly that at least one metallic halide could be formed into a preshaped member and reduced under specific conditions to provide a coherent metallic member. These specific conditions require that the metallic halide be subjected to a stream of gas, the essential active reducing ingredient of which is hydrogen. It is also necessary to employ a temperature range where the reduction of the halide tends to occur to a significant extent. I found further that the preshaped halide member must be heated to a temperature in a temperature range having a lower limit determined by the hydrogen halide partial pressure to the hydrogen partial pressure ratio in equilibrium with the metal of the member and with the member in a range from 0.001 to 0.01. I found also that the upper temperature limit is a range determined by the metallic halide vapor pressure multiplied by the number of halide atoms per metallic atom in a range from 0.001 to 0.01. Under these conditions, I discovered that a preshaped metallic halide member could be formed into a coherent metallic member.

I discovered further that a mixture of metallic halides could also be formed into a preshaped member and reduced under the above conditions to provide a coherent metallic member. For example, such a halide mixture would include the mixing of at least two metallic halide powders such as nickel chloride and chromium trichloride to provide a mixture which is subsequently formed into a preshaped member. The resulting coherent metallic member is a nickel-chromium alloy. The subject method is also applicable to forming at least one mixed metallic halide into a preshaped member which is reduced subsequently under the above conditions to provide a coherent metallic member. Such a mixed halide would include at least two metallic components in the halide, such as nickel and cobalt.

At least one metallic halide and a metal which will react with the metal reduced from the metallic halide are also formed into a preshaped member as disclosed above and reduced to a coherent metallic member. In the formation of such a preshaped member, at least one metallic halide, a mixture of metallic halides or at least one mixed metallic halide is employed. The reacting metal can be a single metal, a metal mixture, or a metallic alloy, or derived from a metal compound, a metal compound mixture, or a mixed metal compound. For example, a nickel halide,  $\text{NiCl}_2$ , and a copper halide,  $\text{CuCl}$ , comprising a mixture of metallic halides and a reacting metal zirconium in the form of zirconium hydride powder are formed together into a preshaped member which is reduced in the manner described above. A reacting metal in the form of a metallic alloy such as an iron-tungsten-carbon alloy in powder form and a mixture of metallic halides of nickel chloride, ferrous chloride, chromium chloride, and cobalt chloride are formed together into a preshaped member.

The coherent metallic member which is formed from the preshaped member is a nickel-iron-chromium-cobalt-tungsten-carbon alloy.

I found further that at least one inert metallic filler or at least one inert non-metallic filler can be combined with at least one metallic halide to form the preshaped member. Furthermore, I found that such a metallic or non-metallic filler could be combined with at least one metallic halide and at least one other reacting metal to form a coherent metallic member. For example, a metallic 10 filler of molybdenum in powder form is mixed with a metallic halide such as a copper chloride to produce a coherent metallic member of copper metal with molybdenum particles therein. A non-metallic filler of magnesium silicate powder is combined with a mixture of metallic halides of nickel chloride and chromium chloride to form upon subsequent reduction a nickel-chromium alloy with magnesium silicate particles therein. A non-metallic filler of titanium oxide powder is combined with a metal compound of titanium hydride and with a mixture 20 of metallic halides of ferrous chloride, nickel chloride, and cobalt chloride to form an iron-nickel-cobalt-titanium alloy with titanium oxide particles therein.

In the single figure of the drawing, the standard free energy of formation of metallic chlorides per mole of chlorine in kilocalories is plotted against temperature in degrees centigrade.

Broken lines 10 and 11 set forth a range for the minimum standard free energy of formation of metallic chlorides per mole of chlorine in kilocalories which is necessary for each of the metallic chlorides set forth on the graph to be reduced to its respective coherent metal at a hydrogen pressure of one atmosphere. Broken lines 10 and 11 define a lower temperature limit determined by the hydrogen chloride partial pressure to the hydrogen partial pressure ratio in equilibrium with the metal of the member and with the member in a range from 0.001 to 0.01. On each line identifying a particular metallic chloride, a point 12 defines the temperature at which the vapor pressure of the metallic chloride multiplied by the number of chlorine atoms per metal atom is equal to 0.001. A point 13 on each line defines the temperature at which the vapor pressure of the metallic chloride multiplied by the number of chlorine atoms per metal atom is equal to 0.01. The metallic chlorides for which points 12 and 13 are plotted to the right and above the lower temperature limit range are reducible to their respective coherent metals without undue loss of metal by evaporation of metallic chloride. The metallic chlorides whose points 12 and 13 are plotted to the left and below the lower temperature limit range are not reducible. Thus, it is feasible to reduce silver chloride, cuprous chloride, nickel chloride, cobalt chloride, ferrous chloride and chromium chloride to their respective coherent metals. It is not feasible to reduce cadmium chloride, zinc chloride or manganese chloride to their respective coherent metals. In the latter metallic chlorides, chloride evaporation occurs more rapidly than reduction of the metal by hydrogen.

While the subject graph sets forth a plurality of metallic chlorides which are suitable in the present method, similar graphs can be prepared for suitable metallic bromides and metallic iodides. When a mixture of metallic chlorides, or a mixed metallic chloride which may be combined with a reacting metal, or a filler or both, to provide a coherent metallic member, a temperature is selected from the above graph which temperature is within the respective temperature range for reduction of the individual metallic chlorides. It is preferred also to reduce the particular chloride or chlorides at a higher temperature within the temperature range to reduce the reduction time.

In accordance with the practice of the present invention, a coherent metallic member of nickel was produced from nickel chloride powder which was formed into a one-quarter inch tablet by pressing at 2000 pounds per

70 square inch. The preshaped nickel chloride tablet was positioned within a chamber. Hydrogen gas was introduced into the chamber at a pressure of one atmosphere and the preshaped metallic chloride was heated to a temperature of 600° C., over a period of seventy minutes. The gas stream and heat were then discontinued and the apparatus was allowed to cool to room temperature. It will be noted from the single figure of the drawing that a minimum temperature of about 190° C. could have been selected to reduce the preshaped nickel chloride member to nickel. It is more desirable from an economic standpoint to employ a higher temperature for the reduction of the metallic chloride thereby reducing the reduction time. While hydrogen gas was employed as the reducing agent, other gas streams can be used provided the essential active reducing ingredient of such a stream is hydrogen.

5 15 20 25 30 35 40 45 50 55 60 65 70 75 Several examples of methods of forming coherent metallic members in accordance with the present invention are as follows:

#### Example I

Nickel chloride powder was formed into a preshaped one-quarter inch tablet by pressing at 2000 pounds per square inch and was positioned within a chamber into which was introduced hydrogen gas at a pressure of one atmosphere. The preshaped metallic chloride was heated to a temperature of 600° C. over a period of seventy minutes. The heat was then discontinued and the apparatus was allowed to cool to room temperature. The coherent nickel member was 14 percent of theoretical density. Subsequently, the nickel tablet was sintered at a temperature of 1350° C. for a period of ten minutes in a hydrogen atmosphere. The member was then 62 percent of theoretical density.

#### Example II

30 35 40 45 50 55 60 65 70 75 Thirty grams of nickel chloride powder and 10.5 grams of chromium trichloride powder were mixed together and pressed into the shape of a bar at a pressure of 2000 pounds per square inch. This preshaped bar was then placed into a chamber into which hydrogen gas was introduced at a pressure of one atmosphere. The bar was heated to a temperature of 600° C. over a period of eighty minutes. It was then heated to 1100° C. for five minutes and heated to 1350° C. for ten minutes. The heat was then discontinued and the apparatus was allowed to cool to room temperature. A coherent nickel-chromium alloy bar of 20 weight percent chromium and 80 weight percent nickel was produced by this method. The bar showed approximately 50 percent linear shrinkage.

#### EXAMPLE III

55 60 65 70 75 A mixture of nickel chloride powder and chromium trichloride powder and an inert non-metallic filler of magnesium silicate were mixed together to give 40 volume percent filler and preshaped into the form of a bar by pressing at 2000 pounds per square inch. The preshaped member was positioned in a chamber into which hydrogen gas was introduced at a pressure of one atmosphere. The preshaped member was heated to a temperature of 600° C. over a period of 80 minutes. It was then heated to 1100° C. for five minutes and heated to 1350° C. for ten minutes. The heat was then discontinued and the apparatus was allowed to cool to room temperature. A coherent nickel-chromium alloy bar of 20 weight percent chromium and 80 weight percent nickel was produced by this method in which magnesium silicate particles were dispersed throughout the volume of the bar.

While other modifications of this invention and variations of method which may be employed within the scope of the invention have not been described, the invention is intended to include such that they may be embraced within the following claims.

What I claim as new and desire to secure by Letters Patent of the United States is:

1. A method of forming a coherent metallic member which comprises forming at least one metallic halide powder into a preshaped powder member, positioning said preshaped member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

2. A method of forming a coherent metallic member which comprises forming a mixture of metallic halide powders into a preshaped powder member, positioning said preshaped member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in the range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

3. A method of forming a coherent metallic member which comprises forming at least one mixed metallic halide powder into a preshaped powder member, positioning said preshaped member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

4. A method of forming a coherent metallic member which comprises forming at least one metallic halide powder and at least one powder containing a metal adapted to form an intermetallic compound with the metal reduced from the metallic halide into a preshaped powder member, positioning said preshaped member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

5. A method of forming a coherent metal which comprises forming at least one metallic halide powder and at least one inert metallic filler into a preshaped powder member, positioning said preshaped member within a chamber, introducing into said chamber a stream of gas, consisting essentially of hydrogen, and heating said member to a temperature in a temperature range having a

lower limit in a range determined by the hydrogen halide partial pressure to the hydrogen partial pressure ratio in equilibrium with the metal of said member and with said member in a range from 0.001 to 0.01 and an upper limit in a range determined by the metallic halide vapor pressure multiplied by the number of halide atoms per metallic atom in a range from 0.001 to 0.01 whereby said member is reduced to a coherent metallic member.

6. A method of forming a coherent metallic member which comprises forming at least one metallic halide powder and at least one inert non-metallic filler into a preshaped powder member, positioning said preshaped member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

7. A method of forming a coherent metallic member which comprises forming at least one metallic halide powder, at least one reacting metal, and at least one inert metallic filler into a preshaped powder member, positioning said member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

8. A method of forming a coherent metallic member which comprises forming at least one metallic halide powder, at least one reacting metal, and at least one inert non-metallic filler into a preshaped powder member, positioning said member within a chamber, introducing into said chamber a stream of gas consisting essentially of hydrogen, and heating said member to a temperature in a temperature range having a lower limit in a range determined by the hydrogen halide partial pressure to the hydrogen partial pressure ratio in equilibrium with the metal of said member and with said member in a range from 0.001 to 0.01, and an upper limit in a range determined by the metallic halide vapor pressure multiplied by the number of halide atoms per metallic atom in a range from 0.001 to 0.01 whereby said member is reduced to a coherent metallic member.

#### References Cited by the Applicant

##### UNITED STATES PATENTS

- |           |         |                 |
|-----------|---------|-----------------|
| 2,418,148 | 4/1947  | Williams et al. |
| 2,663,663 | 12/1963 | Crowley.        |
| 2,664,352 | 12/1953 | Darner.         |

##### FOREIGN PATENTS

- |         |         |                |
|---------|---------|----------------|
| 551,859 | 6/1957  | Canada.        |
| 644,813 | 10/1950 | Great Britain. |
| 668,544 | 3/1952  | Great Britain. |

70 LEON D. ROSDOL, Primary Examiner.

R. L. GRUDZIECKI, Assistant Examiner.